

## UNITED STATES PATENT OFFICE

EMERSON K. LEWIS AND EUGENE WENZ, OF PITTSBURGH, PENNSYLVANIA

## CAST IRON ROLL

No Drawing.

Application filed March 29, 1929. Serial No. 351,116.

The invention relates to iron rolls, and especially to condensed grain cast iron alloy rolls for use in rolling mills. The metal rolling art has long sought an iron roll which possesses the combination of adequate strength, satisfactory surface hardness and suitable grain structure, and which possesses high enough interior hardness to permit substantial dressing and grooving. Rolls as produced at present are generally made from a high carbon iron, and usually contain other hardening elements. The requisite surface hardness is obtained by suitably adjusting the composition, or by casting against heavy chilling rings to obtain a hard, white iron outer chilled portion. However, whether cast against heavy chills, or against lighter chills to produce the so-called condensed grain rolls, the prior rolls have suffered from the serious disadvantage that the interior, unchilled portion is considerably softer than the outer, chilled portion. Furthermore, and what is more serious, the inner zone becomes progressively and rapidly softer toward the center.

As a result of the hardness differential between the outer and inner zones and within the inner zone, the rolls which have been produced heretofore have not been satisfactory because they must be discarded as soon as they are turned down through the hard outer portion. This is especially true of grooved rolls used for rolling shapes or structural forms. As soon as the roots of the grooves penetrate into the softer portion of a roll, it has to be discarded, because the inner, softer portions are not hard enough or sufficiently resistant to wear to permit further use.

An object of the invention is to provide a condensed grain cast iron roll having an outer condensed and an inner uncondensed portion, a close-grained gray iron structure from surface to center, and having a low hardness differential from surface to center.

Another object is to provide a condensed

grain roll of the type referred to in which the condensed portion merges gradually into the uncondensed portion, and in which the hardness of the uncondensed portion is substantially uniform to the center.

A further object is to provide a condensed grain cast iron roll having a close-grained gray iron structure from surface to center irrespective of the degree of chilling, and having high interior as well as surface hardness.

Still another object is to provide a condensed grain cast iron roll relatively low in carbon, having a close-grained gray iron structure from surface to center in which the condensed outer portion merges gradually into the inner uncondensed portion, and in which the hardness of the interior portion is substantially uniform to the center.

Other objects are to provide a condensed grain cast iron roll having a close-grained gray iron structure from surface to center irrespective of the degree of chilling, which is low in carbon and contains substantial amounts of chromium and nickel, and which is especially adapted for use in rolling shapes.

In accordance with the invention the rolls are made from a cast iron alloy containing relatively low amounts of carbon together with substantial amounts of nickel, chromium, and silicon, by casting the iron alloy to form outer condensed and inner uncondensed portions. Preferably, they are cast against the light chills used in making condensed grain rolls. The rolls thus formed have a close-grained gray iron structure from surface to center, and the condensed portions merge gradually into the uncondensed portions. A particular characteristic of these rolls is that the hardness and graphitic carbon content of the uncondensed portion is substantially uniform up to the center; also they possess a very low hardness and graphitic carbon differential from sur-

face to center. Although the invention preferably embodies condensed grain rolls, it is a characteristic of the cast iron alloys used in the practice of the invention that, even when cast in very heavy chills the rolls still possess a gray iron structure from surface to center, the characteristics of which are likely those numerated above.

The iron alloy used in the invention is characterized by a low carbon content relative to that commonly used in cast irons, and it contains a somewhat higher amount of chromium than is usual in a cast iron used for rolls, together with substantial amounts of softening elements such as silicon, and hardening elements such as manganese and nickel, as well as other metals and metalloids, for example, sulfur and phosphorus. In these alloys the carbon may vary from about 2.0 to 3.4 per cent, the higher ranges within these limits being preferred for most purposes. Silicon, which exerts its well known effects, ranges from about 1.25 to 3.0 per cent. This element will be varied in the well understood manner, in accordance with the characteristics desired in the roll, its size, degree of chill, and the like. In general, from about 0.4 to 1.0 per cent of manganese may be used. Chromium, which is used for its hardening effect to compensate for the reduction in carbon, may range from about 0.80 to 2.5 per cent, and preferably from about 1.3 to 2.5 per cent. The nickel content of the alloys may be varied within rather wide limits, from about 0.4 to 3.0 per cent. Manganese and chromium tend to prevent the formation of graphitic carbon, and may for this reason be termed carbon-retaining elements. The alloys may contain about 0.04 to 0.09 per cent of phosphorus. This element, however, is not always easy to control in cast irons, and small variations are permissible. The sulfur is kept low, but for best results is present in an amount greater than about 0.03 per cent.

Rolls thus made in accordance with the invention have a gray iron structure throughout, which is close and fine-grained entirely to the center, and which possesses characteristics novel in such rolls which make them superior for certain purposes to prior rolls. The condensed portion of the rolls merges gradually into the uncondensed portion, and there is no distinct line of demarcation between them. As a matter of fact, it is difficult to determine by visual examination of a fractured or cut groove surface, where the chilled portion ends. This structure is of advantage, because it eliminates sudden changes in physical properties. The graphitic carbon is present in finely divided form, and the grain texture is distinctly that of condensed grain rolls. There is this difference as compared with prior rolls: In those heretofore made, the graphitic carbon content increases

quite sharply in passing inwardly from the surface into the chilled zone, with the result that the rolls are much softer and weaker at the juncture of that zone with the inner, unchilled zone. Furthermore, going inwardly toward the center through the unchilled zone, the graphitic carbon increases gradually, and generally as the center is approached the structure becomes mottled and porous because of the high amount of graphitic carbon. Thus the inner portions of the prior rolls become progressively softer and weaker. These characteristics are decidedly disadvantageous, chiefly because the amount the roll could be turned down (and consequently its useful life) is limited to the depth of the outer, chilled portion. Especially is this a disadvantage in the case of grooved rolls.

In the rolls provided according to this invention the graphitic carbon increases somewhat, but to an appreciably lesser extent than in prior rolls, in passing from the surface to the end of the condensed portion; and what is especially important, the graphitic carbon content from the end of the condensed portion to the center of the roll is uniform, or substantially uniform. Owing to the composition of the rolls and their casting behavior, the surface hardness is high, and this combined with the texture of the grain makes these rolls suitable for roughing or intermediate rolling. The hardness, in consequence of the foregoing properties, does not decrease as much as in prior rolls in passing inwardly toward the center, there being a relatively low hardness differential between the surface and the end of the condensed zone, and the hardness of the uncondensed portion is relatively uniform up to the center. The rolls according to the invention are thus admirably adapted for rolling shapes and structural forms, because the interior of the roll is hard enough and of sufficiently uniform hardness to permit cutting the grooves or tongues well into the roll.

While the preferred practice of the invention is to form condensed grain rolls, they may be cast against the massive chilling rings used to make chilled rolls. In such cases also the rolls possess a gray iron structure throughout, which is similar in appearance and properties to that described hereinabove, the properties being modified in the manner to be expected from severe chilling. Thus it will be understood that the property of securing a roll having condensed and uncondensed portions of gray iron merging one into the other and in which there is a low hardness differential from surface to center and particularly in the uncondensed zone, is a characteristic of the invention irrespective of the degree of chilling.

In general it may be said that where great toughness is desired, for rolls subject to se-

vere shock, the lower ranges of composition given will be used. Rolls made from the higher ranges are in general less tough, but of greater hardness, and possess high wear resistance. Properties intermediate these may be secured by suitable selection of the alloy components.

The following actual example illustrates the important advantages of the invention.

10 A cast iron alloy selected to give medium hardness with a desirable combination of toughness and strength and containing about 3.17 per cent of carbon, 1.75 per cent of silicon, 0.57 per cent of manganese, 1.35 per cent 15 of chromium, 0.52 per cent of nickel, 0.038 per cent of sulfur, and 0.097 per cent of phosphorus was cast in the form of a roll having a body  $22\frac{3}{4}$  inches in diameter and 27 $\frac{1}{2}$  inches long, with necks 13 $\frac{3}{8}$  inches in 20 diameter and 14 inches long. The roll was cast against light chilling rings to give the condensed grain structure. A transverse slice 1 $\frac{1}{8}$  inches wide was cut from the center of the roll body, and holes  $\frac{3}{2}$  inches in diameter were drilled 1 inch apart from center to center across a diameter of this section, the turnings from each hole being segregated for analysis. Scleroscope hardness tests were also made on this section, along a diameter thereof. The results are shown in the following table, each figure being the average of corresponding diametrically opposed points:

| Distance from surface | Graphitic carbon | Scleroscope | Inches   |          |
|-----------------------|------------------|-------------|----------|----------|
|                       |                  |             | Per cent | Hardness |
| $\frac{1}{2}$         | 1.71             | 46.1        |          |          |
| 1                     | 1.86             | 44.2        |          |          |
| 2                     | 1.86             | 42.6        |          |          |
| 3                     | 1.91             | 41.4        |          |          |
| 4                     | 1.97             | 40.1        |          |          |
| 5                     | 1.86             | 40.3        |          |          |
| 6                     | 1.94             | 39.6        |          |          |
| 7                     | 1.96             | 39.5        |          |          |
| 8                     | 1.99             | 38.6        |          |          |
| 9                     | 1.99             | 38.6        |          |          |
| 10                    | 1.94             | 38.2        |          |          |

These data show that, within the limits of experimental error, the graphitic carbon content and the hardness remain substantially constant from a point about three inches from the surface up to the center, and that from the surface, or close to the surface, to the center, there is but a low graphitic carbon and hardness differential, i. e., the inner and outer zones approximate each other in hardness. They show further that in this roll the difference in hardness between the outer condensed portion and the inner uncondensed portion is only 8 points, which is so low that 55 rolls according to the invention can be cut down to an extent which has heretofore been impossible.

Tensile and transverse test bars were cut from the periphery of the roll body, the 60 average tensile strength being 27250 pounds

per square inch, and the average of the transverse or bending tests being 3942 pounds per square inch, the supports in these tests being spaced 10 $\frac{1}{2}$  inches apart. Tensile test bars were cut from the transverse body section 70 used for the hardness tests and carbon analyses. These showed strengths of about 25000 pounds per square inch at 3 inches from the surface, and from there inwardly to the center the strength averaged about 20000 75 pounds per square inch.

As further showing the properties to be independent of the degree of chilling, the drag neck, which was of course cast in sand, was sectioned 6 $\frac{1}{2}$  inches from the body, and turnings for analysis taken as before, which showed the graphitic carbon content to be substantially constant from a point about 1 inch from the surface to the center. The data are given in the following table:

| Distance from surface | Graphitic carbon |
|-----------------------|------------------|
| Surface               | Per cent         |
| 1                     | 1.79             |
| 2                     | 2.0              |
| 3                     | 1.9              |
| 4                     | 1.87             |
| 5                     | 1.82             |
| 6                     | 1.89             |
| Center                | 1.93             |

As further illustrative of the benefits of the invention, the following data obtained from another roll cast and tested as in the preceding example are cited. The body of 103 this roll was 42 inches in length and 30 $\frac{3}{4}$  inches in diameter, and the necks were 19 $\frac{1}{2}$  inches long and 18 $\frac{1}{8}$  inches in diameter. The average analysis of drillings taken across the body as in the case of the preceding roll was 105 as follows:

|                 | Per cent |
|-----------------|----------|
| Total carbon    | 2.80     |
| Combined carbon | 1.15     |
| Manganese       | 0.33     |
| Chromium        | 1.13     |
| Nickel          | 1.60     |
| Silicon         | 1.44     |
| Sulfur          | 0.037    |
| Phosphorus      | 0.065    |

After being turned to a diameter of 30 $\frac{3}{4}$  inches, the surface hardness of the body of this roll, measured with a scleroscope, was 55. The tensile and transverse strengths of 110 test bars cut longitudinally from periphery of the body were 35590 and 4460 pounds per square inch respectively. The supports for the transverse tests were spaced 10 $\frac{1}{2}$  inches. The average tensile strength of bars cut from the transverse body section was 38500 pounds 115 per square inch just below the surface, 36750 pounds per square inch three inches below the surface, and from there inwardly to the center the average strength was 25430 pounds per square inch.

Hardness tests and graphite carbon analyses were made along a diameter of a slice taken from the body, as in the preceding example, the results being as follows:

|    | Distance from surface | Graphitic carbon |          | Scleroscope |
|----|-----------------------|------------------|----------|-------------|
|    |                       | Inches           | Per cent |             |
| 10 | 1/4                   |                  |          | 58.9        |
|    | 1/2                   |                  |          | 55.1        |
|    | 1                     | 1.41             |          | 53.9        |
|    | 2                     | 1.69             |          | 51.2        |
|    | 3                     | 1.67             |          | 48.1        |
|    | 4                     | 1.65             |          | 46.3        |
|    | 5                     | 1.71             |          | 45.1        |
|    | 6                     | 1.70             |          | 43.7        |
|    | 7                     | 1.67             |          | 42.0        |
|    | 8                     | 1.72             |          | 41.5        |
|    | 9                     | 1.67             |          | 43.4        |
|    | 10                    | 1.66             |          | 41.0        |
|    | 11                    | 1.68             |          | 39.4        |
|    | 12                    | 1.64             |          | 39.1        |
|    | 13                    | 1.66             |          | 38.1        |
|    | 14                    | 1.61             |          | 37.7        |
|    | 15 1/4 (Center)       | 1.69             |          | 36.6        |

As in the case of the first-cited roll, the graphitic carbon is practically constant from the end of the condensed outer portion to the center of the roll. In this case the condensed portion extended about four inches into the roll. Likewise, the hardness differential from the beginning of the uncondensed portion to the center is very low. And all of the advantages previously discussed were present in both rolls.

Analysis of the rolls made across a diameter of the body and of the neck show, in addition to the foregoing characteristics, that there is substantially no tendency toward segregation of any of the elements, even in very large rolls. This is, of course, of great advantage.

The invention provides condensed grain rolls which from all standpoints overcome the disadvantages of prior rolls. These rolls possess condensed and uncondensed portions which merge gradually into one another, which approximate one another in hardness, and which are of a fine grain throughout. The interior uncondensed portions possess a uniformity of hardness hitherto unobtainable, and these properties make the normal life of the rolls very great, because not only is their strength sufficiently high, but they may be turned down or grooves cut deeper into the uncondensed portions than was previously possible, with fully adequate strength, interior hardness and resistance to wear.

According to the provisions of the patent statutes, we have explained the principle and mode of operation of our invention, and have described what we now consider to represent its best embodiment. However, we desire to have it understood that, within the scope of the appended claims the invention may be practiced otherwise than as specifically described.

We claim as our invention:

1. As a new article of manufacture, a condensed grain cast iron roll formed of an iron

alloy containing about 2 to 3.4 per cent of carbon, about 0.8 to 2.5 per cent of chromium about 0.4 to 3.0 per cent of nickel, about 1.25 to 3.0 per cent of silicon, and about 0.4 to 1.0 per cent of manganese, proportioned to provide a close grained gray iron structure from surface to center irrespective of the degree of chilling, and having outer condensed grain and inner uncondensed portions, a low hardness differential from surface to center, and substantially uniform hardness in said uncondensed portion.

2. As a new article of manufacture, a condensed grain cast iron roll formed of an iron alloy containing about 2 to 3.4 per cent of carbon, about 1.3 to 2.5 per cent of chromium, about 2.5 per cent of silicon, about 0.4 to 3 per cent of nickel, and about 0.4 to 1 per cent of manganese, proportioned to provide a close grained gray iron structure from surface to center irrespective of the degree of chilling, and having outer condensed grain and inner uncondensed portions, a low hardness differential from surface to center, and substantially uniform hardness in said uncondensed portion.

In testimony whereof, we hereunto sign our names.

EMERSON K. LEWIS.  
EUGENE WENZ.

70

75

85

90

95

100

105

110

115

120

125

130